

H. R. WARDELL.  
MANUFACTURE OF ASPHALT.  
APPLICATION FILED AUG. 30, 1919.

1,385,511.

Patented July 26, 1921.

Fig. 1.



Fig. 2.



# UNITED STATES PATENT OFFICE.

HENRY R. WARDELL, OF NEW YORK, N. Y., ASSIGNOR TO CENTRAL COMMERCIAL COMPANY, OF CHICAGO, ILLINOIS, A CORPORATION OF ILLINOIS.

## MANUFACTURE OF ASPHALT.

1,385,511.

Specification of Letters Patent. Patented July 26, 1921.

Application filed August 30, 1919. Serial No. 320,906.

To all whom it may concern:

Be it known that I, HENRY R. WARDELL, a citizen of the United States, and resident of New York city, county and State of New York, have invented certain new and useful Improvements in the Manufacture of Asphalt, of which the following is a specification, and which are illustrated in the accompanying drawings, forming a part thereof.

The invention relates to the manufacture of asphalts from petroleum residuum, and to the resulting products; the object of the invention being to improve such manufacture and products, having particular reference to asphalts for roofing and paving purposes of the nature of those heretofore obtained by the mixing of a mineral bitumen known as grahamite with residuum from Mexican petroleum.

It is well known that petroleum residuum may be oxidized by treatment with air, in accordance with the method disclosed in the now expired patent to Culmer, No. 635,429, dated October 24, 1899, and that asphaltic fluxes or so-called blown oil asphalts are thereby produced. But these asphaltic fluxes, whether produced by the said treatment of residuum from mid-continent mixed base petroleum residuum, or of residuum from Mexican or California asphaltic base petroleum, are not satisfactory for roofing and paving purposes except when compounded with natural asphalts, such as Trinidad asphalt, gilsonite, elaterite, and the like. While residuum from mid-continent crude petroleum may be so oxidized as to produce an asphaltic flux having the high melting point required in asphalts for roofing and paving purposes, this product lacks ductility and strength. On the other hand, residuum from Mexican or California petroleum, being originally low in its petroleo content, is not capable of oxidation to a point where the desirable high melting point is obtained in the resulting product.

These blown oil asphalts must, therefore, be compounded with more expensive materials for the purpose of improving ductility when mid-continent residuum has been used, and for the purpose of raising the melting point when Mexican or California residuum has been used. Compounding either of the said two kinds of blown oil asphalts with

the other when the two have been separately prepared does not produce a satisfactory product.

As oxidation of petroleum residuum by the said air treatment is understood to result in the conversion of petroleo into asphaltene, and as a high melting point in the product is only obtained when mid-continent or other residuum containing relatively large amounts of petroleo is used, it seems to follow that the asphaltene produced by this oxidation is not the same in all respects as the asphaltene which constitutes the principal constituent of Mexican and California residuums, but has a higher melting point. It is found, however, that by first compounding a mixed base residuum, such as that obtained from mid-continent petroleum, with asphaltic base residuum obtained from Mexican or California petroleum and then oxidizing the said mixed residuums with air, an asphalt is produced which is markedly different from the blown asphalts obtained by the separate treatment of either of the said residuums as well as from any compound of the said blown oil asphalts, and is useful for roofing and paving without the addition thereto of natural asphalts.

The present invention accordingly contemplates the improved method of manufacturing asphalt, which consists in first compounding mixed base petroleum residuum and asphaltic base petroleum residuum with each other and then "blowing" the resulting compound and the new asphalt so produced.

Apparatus to be used in practising the said improved method may take the form illustrated in the accompanying drawings, wherein

Figure 1 is a central longitudinal sectional view of a retort equipped with the required air induction pipes and the associated furnace; and

Fig. 2 is a detail transverse sectional view taken on line 2—2 of Fig. 1, but drawn to a larger scale.

The retort 10 is illustrated as being of cylindrical form, horizontally arranged in the furnace setting, generally designated 11. It is equipped with normally covered manholes 12, 13, for the introduction of the charge, a draw-off pipe 14 controlled by valve 15, and vent pipe 16. The furnace

setting 11 is constructed to provide a firebox 17, to which a portion of the under side of the retort 10 adjacent one end of the same is directly exposed, and flues 18, 19, leading rearwardly under the retort to its opposite end and then forwardly along the opposite sides of the retort and downwardly to a smoke tunnel 20. An air blast pipe 21 extends longitudinally over the retort at one side of the same for connection with each of a series of branches 22, which enter the retort 10 at short intervals throughout its length and reach nearly to the bottom of the same.

15 As an example of the practice of the improved method embodying the present invention a mixture of Mexican residuum of 8° to 10° Bé., and Illinois residuum of 12° to 14° Bé., comprising 60% by weight of the former and 40% by weight of the latter, may be placed in the retort 10 and brought to a temperature of 450° F. While approximately this temperature is maintained, air is introduced through the blast pipe 21 and branches 22 at the rate of ten unit volumes of air per minute for each unit volume of the mixed residuums contained in the retort until the charge is of such consistency that it will solidify when allowed 25 to cool. The product has physical properties resembling the compound produced by "cutting" grahamite obtained at Sardis, near Tuskaoma, Pushmataha county, Oklahoma, with Mexican flux oil, and may be used 30 for roofing or paving without being compounded with other asphalts.

Although some variation in temperature during the treatment can scarcely be avoided, it has been found that if the treatment be 35 continued for a period of seventy-two hours without variation of the temperature beyond the limits of 450° F. and 500° F., the said product will be characterized by showing a penetration of twenty points with the 40 Howard and Morse penetrometer at 77° F. and ten points at 32° F., a ductility of 8 to 10 centimeters with the Dow mold, and a melting point of 275° F. by the ring and ball method. On the other hand, a similar 45 treatment of Illinois residuum of 12° to 14° Bé. for a like period produces an asphalt showing a penetration of twenty points at 77° F., and fifteen points at 32° F., a melting point of 290° F. and no appreciable ductility; while a similar treatment of Mexican 50 residuum for a like period produces an asphalt showing a penetration of twenty points at 77° F., no appreciable penetration at 32° F., ductility of ten to fifteen centimeters, and a melting point of 160° F.

It will thus be seen that while the improved product obtained by the practice of the invention in the manner herein selected as an example has nearly the same melting 55 point as the asphalt obtained by blowing

Illinois residuum, and also shows nearly the same penetration as the latter at both summer and winter temperatures, its ductility compares favorably with that obtained by blowing Mexican residuum.

The mixture of pure asphaltic base petroleum residuum and mixed base petroleum residuum comprising the charge may be substantially varied from the proportions given, 70 25% of the mid-continent residuum and 75% of the Mexican product being useful for some purposes. It may be stated as a rule that the melting point of the asphalt produced varies with the relative amount of the mixed base residuum contained in the 75 charge. That is to say, addition of a larger amount of the mixed base residuum produces more of the petroleenes capable of conversion by oxidation into high melting point asphaltenes. Likewise the temperature of 80 treatment and the rate of blowing may both be varied from the figures given, increase in temperature and rate of blowing both tending to reduce the time of treatment necessary for solidification of the material. 85

While the improved product is preferably produced without the addition of natural asphalt, it will be understood that natural asphalt may be used in the charge if desired, in which case the product will be 90 superior to that produced by blowing either a mixture of mixed base petroleum residuum and natural asphalt, or a mixture of asphaltic base petroleum residuum and natural asphalt. 95

I claim as my invention—

1. The method of manufacturing asphalt which consists in compounding a mixed base petroleum residuum and an asphaltic base petroleum residuum, and then maintaining 10 the said mixed residuums at a temperature above that required for complete expulsion of water vapor but below that of destructive distillation while simultaneously blasting the charge with air until an asphalt which is solid at ordinary temperatures is obtained.

2. The method of manufacturing asphalt which consists in compounding an asphaltic base petroleum residuum and a petroleum 11 residuum containing petroleene in substantial quantity, and then maintaining the said mixed residuums at a temperature above that required for complete expulsion of water vapor but below that of destructive 1 distillation while simultaneously blasting the charge with air until an asphalt which is solid at ordinary temperatures is obtained.

3. The method of manufacturing asphalt which consists in compounding an asphaltic 1 base petroleum residuum of 8° to 10° Bé. gravity and a mixed base petroleum residuum of 12° to 14° Bé. gravity and then maintaining the said mixed residuums at a temperature of about 450° F. while simulta- 1

neously blasting the charge with air until an asphalt which is solid at ordinary temperatures is obtained.

4. The method of manufacturing asphalt which consists in compounding an asphaltic base petroleum residuum of about 8° to 10° Bé. gravity and a mixed base petroleum residuum of about 12° to 14° Bé. gravity in the proportions of about 60 per cent. of the asphaltic base residuum and 40 per cent. of the mixed base petroleum residuum and then maintaining the said mixed residuums at a temperature of about 450° F. while simulta-

neously blasting the charge with air until an asphalt which is solid at ordinary tem- 15 peratures is obtained.

5. The asphalt produced by blasting with air a mixture of asphaltic base petroleum residuum and a petroleum residuum containing petrolene in substantial quantity at a 20 temperature above that required for complete expulsion of water vapor, but below that of destructive distillation until a product which is solid at ordinary temperatures is obtained.

HENRY R. WARDELL.